

## UNITED STATES PATENT OFFICE

HARRY W. TURNER, OF SCHENECTADY, NEW YORK, ASSIGNOR TO GENERAL ELECTRIC COMPANY, A CORPORATION OF NEW YORK

METHOD OF MAKING TEXTILE MATERIAL PERMANENTLY FLEXIBLE, WEATHERPROOF, AND FIRE RESISTANT

No Drawing.

Application filed March 25, 1932. Serial No. 601,304.

The present invention relates broadly to a method of treating textile materials and is more specifically concerned with a simple method whereby textile material, for example, canvas, is treated so that it is permanently flexible in character, dust proof and resistant to fire and weather.

In the construction of electrical apparatus the need often arises for flexible insulation embodying textile material. Textile material, such as canvas, has heretofore been employed for the purpose, but difficulties have arisen in that the material was not fire-proof and especially susceptible to fire from sparks generated in or near the electrical apparatus. The material was therefore treated to render it less inflammable but usually such treatment was not only expensive but in addition did not give a permanently flexible product.

In accordance with my discovery I have effected a simple process whereby I can easily and economically treat textile fabrics in order to render them permanently flexible, dust proof, weather resistant and fire resistant, especially from sparks, without impairing, and in fact, enhancing the insulation value of the material.

In order that my invention may be better understood and practiced by those skilled in the art to which it pertains I shall describe the process I employ more in detail.

Suitable textile material, for example, 12-ounce duck is first singed on both surfaces. Powdered filling material, for example, talc or soapstone is then incorporated therewith, for instance, by rubbing and kneading it into the pores of the material. This fills in the cellular air spaces in the material rendering it air tight and substantially non-inflammable and supplies in addition a dry lubricant to the material. The treated material is now immersed in and thoroughly impregnated with degelled oil which, as is known, is oil which has been caused to reliquify by heat after having previously been gelled; for example, the material is soaked in degelled linseed oil varnish for about 10 minutes. The degelled oil binds all of the components together and renders the product permanently flexible in character. The material is then

drained and air dried for about 24 hours, after which more powdered talc or soapstone is rubbed and kneaded into the pores of the material.

The product obtained by the above treatment has been found to be excellent in prolonged service tests as regards flexibility, non-inflammability and weather resistant qualities.

What I claim as new and desire to secure by Letters Patent of the United States, is:

A method for treating textile material which consists in singeing the surfaces thereof, incorporating powdered talc into the pores thereof, impregnating the material so treated with degelled linseed oil, air drying the material and again incorporating powdered talc therewith.

In witness whereof, I have hereunto set my hand.

HARRY W. TURNER.

70

75

80

85

90

95

100